

# United States Patent Office

3,189,497

Patented June 15, 1965

1

3,189,497

**BORON HYDRIDE SALT-HYDRAZINE SYSTEM**  
Robert E. Williams, La Canada, Calif., assignor to National Engineering Science Co., Pasadena, Calif., a corporation of California  
No Drawing. Filed Mar. 29, 1962, Ser. No. 183,392  
13 Claims. (Cl. 149—22)

The present invention relates to a reaction system or mixture of the type used to provide the propulsive force for rockets, missiles, etc.

Countless materials have been proposed and tested as propellants, but very few have been found to possess, to a sufficient degree, the properties essential for operability. One of the principal difficulties encountered by prior workers in this area has been the variation in the pressure and heat generation of the materials tested. Aside from the disadvantage of nozzle erosion due to such variations, the explosive nature of the materials (which is, of course, a necessary property of propellants) often resulted in variations so violent that the rocket was destroyed. Alternatively, the reaction may follow a path leading to undesirable by-products which in turn would reduce the theoretically available energy.

An important feature of the present invention is that it provides a reaction system or mixture containing an additive which moderates the pressure and heat generation of the reaction system or mixture such that it will be sufficiently constant to permit the use of the reaction system or mixture as a rocket or missile fuel.

Another important feature of the present invention is that the substance added to the reaction system or mixture has, itself, propulsive properties.

Briefly stated, the present invention comprises the addition of a lithium borane,  $\text{LiB}_4\text{H}_7$ , or the combination of this lithium borane with hydrazine or the combination of  $\text{LiB}_4\text{H}_7$  with pentaborane-9,  $\text{B}_5\text{H}_9$ , to a reaction system or mixture comprising pentaborane-9 and hydrazine. The  $\text{LiB}_4\text{H}_7$  is added in amount sufficient to prevent the entire system from exceeding the decomposition temperature threshold of hydrazine.

An object of the present invention is to provide a reaction system or mixture which does not generate pressure and heat so violently that destructive explosions occur.

Another object of the present invention is to provide a reaction system or mixture comprising pentaborane-9 and hydrazine which is moderated with an additive such that the hydrazine is prevented from reacting as a monopropellant.

A further object of this invention is to provide a reaction system or mixture comprising pentaborane-9 and hydrazine which is moderated with an additive such that the system is not susceptible to destructive explosions.

A still further object of the present invention is to provide a reaction system or mixture comprising pentaborane-9 and hydrazine which contains, as a moderating additive,  $\text{LiB}_4\text{H}_7$  or  $\text{LiB}_4\text{H}_7$  in combination with pentaborane-9 or hydrazine.

Still another object of this invention is to provide a reaction system or mixture comprising pentaborane-9 and hydrazine which contains, as a moderating additive,  $\text{LiB}_4\text{H}_7$  or the combination of  $\text{LiB}_4\text{H}_7$  and either hydrazine or pentaborane-9, the additive being present in an amount sufficient to prevent the heat generated by reaction of the system from reaching the decomposition temperature threshold of hydrazine.

Other objects and advantages of the present invention, it is believed, will be readily apparent from the following description thereof.

A mixture of pentaborane-9 and hydrazine is believed to function desirably as a propellant combination when

5

15

20

25

30

35

40

45

50

55

60

65

70

2

the reaction of these materials can be controlled such that it is in accordance with the equation:



However, it is also believed that an intermediate reaction occurs according to the equation:



when pentaborane-9 and hydrazine are reacted.

The intermediate reaction designated Equation 2 is believed to be highly detrimental in that the heat of reaction thereof is believed to be sufficiently high that it exceeds the decomposition temperature threshold of hydrazine. This would, of course, result in reaction of the hydrazine as a monopropellant, which reaction does not generate as much propulsive force as the reaction with pentaborane-9. Moreover, some pentaborane-9 is thereby left unreacted and is wasted. By this mechanism the efficiency of the overall system declines and the pentaborane-hydrazine system becomes inefficient to a degree such that it is rendered commercially undesirable. Furthermore, the reaction could proceed in such a manner that control of the hydrazine-pentaborane-9 reaction would be lost and destructive explosion would occur. The occurrence of intermediate Reaction 2 would be consistent with the reaction of pentaborane-9 and tri-methyl-amine reported, by Hough, Ford and Edwards, in "Abstracts of the 135th American Chemical Society Meeting, Boston, April (1959)," as producing the  $\text{B}_4\text{H}_6$ :trimethylamine adduct.

Because of the instability caused by intermediate Reaction 2, the hydrazine-pentaborane-9 system has not heretofore been successfully used as a propellant combination. Were it not for this instability, the high specific impulse of the hydrazine-pentaborane-9 system would make it highly suitable as a propellant combination.

The present invention contemplates the addition of  $\text{LiB}_4\text{H}_7$  to the hydrazine-pentaborane-9 system to control the heat generated by the system such that the decomposition temperature threshold of hydrazine is not reached.

The salt  $\text{LiB}_4\text{H}_7$  mixes with hydrazine releasing a smaller amount of heat than Equation 2. Furthermore,  $\text{LiB}_4\text{H}_7$  is soluble in pentaborane-9. The reaction of  $\text{LiB}_4\text{H}_7$  and  $\text{N}_2\text{H}_4$  would deliver a large amount of propulsive energy, probably according to the reaction:



Therefore, a combination of the  $\text{LiB}_4\text{H}_7$ -hydrazine system with the hydrazine-pentaborane-9 system in proportions such that a sufficient amount of the former is present to prevent the latter from reaching the decomposition temperature threshold of hydrazine would create a thermodynamic balance such that almost the full potential of the pentaborane-9-hydrazine system would be realized, i.e., the complete mixing occurs at a low enough temperature such as to significantly eliminate the hydrazine reacting as a monopropellant.

For example, the lithium borane system may be added to the pentaborane system in the following manner:

$\text{LiB}_4\text{H}_7$  is mixed with pentaborane-9 in sufficient quantity that a mixture containing four mole percent  $\text{LiB}_4\text{H}_7$  and ninety-six mole percent pentaborane-9 is obtained. The reaction mixture within the scope of the present invention may be obtained by combining this mixture with hydrazine in stoichiometric amounts according to Equations 1 and 3.

The  $\text{LiB}_4\text{H}_7$  used in the present invention may be prepared by the reaction of  $\text{B}_5\text{H}_9$  and  $\text{LiH}$  in ether. This reaction, which also produces  $\text{LiBH}_4$  as a by-product

which may be recycled into the  $B_5H_9$  synthesis, is believed to proceed according to the equation:



It is another feature of this invention that the  $LiB_4H_7$ -hydrazine system has propulsive properties which would permit the use of this system independently as a monopropellant mixture or as a solid-liquid propellant combination.

Because of the solubility of  $LiB_4H_7$  in pentaborane-9, it is preferred to add the lithium borane to the pentaborane-9 phase of the reaction system or mixture. Furthermore, the  $LiB_4H_7$  increases the density of pentaborane-9, thereby increasing the "density impulse" of the system.

The quantitative amount of  $LiB_4H_7$  which is added to the hydrazine-pentaborane-9 system will vary depending on such factors as the efficiency of the mixing jets which determine the probability of local "hot spots," the ambient temperature at which the propellant is fired which depends upon the amount and type of insulation used to encase the propellant, etc. However, as previously mentioned, the qualitative amount of  $LiB_4H_7$  must be sufficient to prevent the heat generated by the system as a whole from reaching the decomposition temperature threshold of hydrazine. More than this minimum amount of  $LiB_4H_7$  may be added without serious detrimental effect.

It will be obvious to one skilled in the art that the systems of the present invention have many possible applications as a fuel and source of propulsive power, particularly in rockets and missiles.

Having fully described the present invention, it is to be understood that it is not to be limited to the details set forth, but is of the full scope of the appended claims.

I claim:

1. A mixture comprising pentaborane-9, hydrazine and  $LiB_4H_7$ .
2. A mixture comprising pentaborane-9, hydrazine and  $LiB_4H_7$ , the  $LiB_4H_7$  being present in an amount sufficient to prevent the heat generated by the reaction of the mixture from causing the hydrazine to react as a monopropellant.
3. A reaction system comprising reactive amounts of

pentaborane-9 and hydrazine, and a reaction moderator comprising  $LiB_4H_7$ .

4. The reaction system of claim 3 wherein the  $LiB_4H_7$  is present in an amount sufficient to prevent the heat generated by the reaction of the system from reaching the decomposition temperature threshold of hydrazine.

5. The reaction system of claim 4 wherein the  $LiB_4H_7$  is present in the pentaborane-9 phase of the system.

6. A reaction system comprising reactive amounts of pentaborane-9 and hydrazine, and a reaction moderator comprising  $LiB_4H_7$ , said moderator being present in the pentaborane-9 phase of the system.

7. The reaction system of claim 6 wherein the pentaborane-9 phase comprises four mole percent  $LiB_4H_7$  and ninety-six mole percent pentaborane-9.

8. A reaction system comprising reactive amounts of pentaborane-9 and hydrazine, and a reaction moderator comprising  $LiB_4H_7$  and hydrazine.

9. The reaction system of claim 8 wherein the reaction moderator is present in an amount sufficient to prevent the heat generated by reaction of the system from reaching the decomposition temperature threshold of hydrazine.

10. A process comprising the step of reacting pentaborane-9 with hydrazine in the presence of  $LiB_4H_7$ , the  $LiB_4H_7$  being present in an amount sufficient to prevent the heat generated by said reaction from reaching the decomposition temperature threshold of hydrazine.

11. The process of claim 10 wherein the  $LiB_4H_7$  is present in the pentaborane-9.

12. The process of claim 11 wherein the  $LiB_4H_7$  is present in the ratio of 4 mole percent to 96 mole percent pentaborane-9.

13. A process comprising reacting pentaborane-9 and hydrazine in the presence of a reaction moderator, said reaction moderator comprising  $LiB_4H_7$  and hydrazine, said reaction moderator being present in an amount sufficient to prevent the heat generated by said reaction from reaching the decomposition temperature threshold of hydrazine.

40 No references cited.

CARL D. QUARFORTH, Primary Examiner.

LEON D. ROSDOL, Examiner.